

## UNITED STATES PATENT OFFICE

2,607,737

## CONDENSATION PRODUCT OF A 2-THIO-THIAZOLE, FORMALDEHYDE, AND ALKYL PHENOL TO INHIBIT SULFUR CORROSIVE LUBRICANTS

Richard L. Woodruff, Richmond, and William T. Stewart and Warren Lowe, Berkeley, Calif., assignors to California Research Corporation, San Francisco, Calif., a corporation of Delaware

No Drawing. Application July 9, 1949,  
Serial No. 103,938

3 Claims. (Cl. 252—47)

1

The present invention relates to lubricating oils compounded with active sulfur-containing compounds, such as metal salts of thiophosphates, which composite oils are severely corrosive to silver and like bearings, and to the prevention of such sulfur attack on silver by incorporating in said severely corrosive compounded oils certain agents, such as a condensation product of 2-mercapto-benzothiazole, formaldehyde and octadecyl phenol.

As is well known, the present-day problems involved in the lubrication of internal combustion engines are extremely complex and difficult to overcome, due mainly to the great loads imposed on bearings; the high engine speeds, and the elevated operating temperatures. To avoid rapid deterioration resulting from such severe operating conditions, lubricating oils have been compounded with various improving or stabilizing agents.

Of the various lubricating oil compounding agents, many of the most effective are compounds containing sulfur. For example, aliphatic polysulfides, metal salts of organo-thiophosphates, etc., are highly effective oxidation inhibitors; and sulfurized olefins, xanthate esters and the like are excellent extreme-pressure agents. Unfortunately, oils compounded with such active sulfur-containing compounds are severely corrosive to silver and like metals. The deleterious action involves a direct attack of the metal by sulfur, resulting in a rapid darkening of the metal surface and formation of sulfides and the subsequent sloughing off of the sulfides during engine operation. Thus, there is a considerable loss of bearing metal and a pitting of bearing surfaces. This sulfur attack may be designated as "sulfur corrosion," as distinguished from corrosion caused by action of acids and peroxides which are found as products of oxidation of lubricating oils, particularly highly-refined lubricating oils. This latter type of corrosion, which may be called "oxidation corrosion," or "acid corrosion," adversely affects such hard metal alloys as cadmium-silver, copper-lead, etc., but does not seriously affect silver or bronze. Such oxidation corrosion is usually minimized by the presence of oxidation inhibitors, which reduce the formation of the corrosive acids and peroxides.

It is apparent that in spite of the long desire to lubricate silver bearings with lubricants compounded with active sulfur compounds, it has been impractical to do so in view of the aforementioned severe corrosivity to silver.

Therefore, it is an object of this invention to

provide a non-silver-corrosive lubricant containing active sulfur compounds.

In the attainment of this object, the present invention concerns a lubricant compounded with active sulfur compounds, which compounded lubricant is severely corrosive to silver, and a combination of silver-protective agents which greatly minimize attack on silver by sulfur in the compounded lubricant but without adversely affecting the desired functioning of the sulfur compounds.

Heretofore, in the lubrication of engines having silver metal wearing surfaces, for example, in certain railroad diesel engines which use silver wrist pin bushings, it has been difficult to prevent sulfur attack of the silver surfaces. Because the silver surfaces (e. g., the silver wrist pin bushings) are susceptible to attack by the sulfur of the sulfur-containing lubricating oil additives, there has been a tendency to eliminate highly effective sulfur-containing additives from the diesel lubricating oils, thereby losing the remarkable benefits of these additives. As noted hereinabove, certain highly effective lubricating oil anti-oxidants contain sulfur, which is corrosive to silver. These effective anti-oxidants have not been used in diesel engines containing silver wrist pin bushings without sulfur attack of the silver. Alternative practices have been to eliminate the sulfur-containing additives from the oil, allowing the oil to deteriorate more rapidly through oxidation; or the sulfur-containing additives have been included in the oil formulation, with the resulting sulfur corrosion of the silver wrist pin bushings. Silver is also used in wearing surfaces in aircraft engines, but because of the presence of the silver, the highly effective sulfur-containing aviation oil additives are not used. Now, however, by using the compounds of this invention, lubricating oils compounded with sulfur-containing additives can be used in diesel oils, aviation oils, and any other oils where sulfur corrosion of metals is a problem.

It is of extreme advantage to use a lubricant composition which is effective not only in inhibiting oxidation corrosion, but which is also effective in preventing sulfur attack on metals. In railroad oils, for example, it has been a handicap to use lubricants which inhibit corrosion resulting from oxidation products but permit unhampered attack on metals by compounds having active sulfur present.

While the outstanding advantages of the cooperative action of the silver protective agents in otherwise severely corrosive lubricants contain-

ing sulfur compounds is particularly apparent in heavy duty motor oils, the invention combination finds application in turbine oils, gear oils, such as for use in hypoid gears, cutting oils, soluble oils, greases, etc.

The action of the silver protective agents cannot be explained on any simple basis, since their apparent effect appears anomalous: On the one hand, the protective agents prevent destructive attack of the sensitive metal by active sulfur compounds; but, on the other hand, they do not interfere with the functioning of extreme pressure agents which are believed to act by reaction with the metal surface.

The silver protective agents of this invention which reduce the sulfur attack on silver are condensation products obtained by reacting together approximately equimolar amounts of a 2-thiazole compound, formaldehyde and an alkyl phenol. That is, the products obtained by reacting together about equimolar amounts of 2-thio-thiazoles, formaldehyde and alkyl phenols are effective in reducing the sulfur attack on silver according to this invention.

The simplest member of the 2-thio-thiazole group is 2-mercaptop-thiazole. Also included are the derivatives of 2-mercaptop-thiazole, wherein there may be substituents in the ring carbon atoms.

In 2-thio-thiazole, the hydrogen atoms of the thiazole ring may be substituted by short-chained saturated and unsaturated radicals (e. g., methyl, ethyl, propyl, butyl, ethenyl, propenyl, butenyl, etc.). It is preferred that the substituents contain a total of not more than 20 carbon atoms.

The two adjacent carbon atoms of 2-thio-thiazole may form part of a benzene ring, such as in 2-mercaptop-benzothiazole. The 2-mercaptop-benzothiazole may be substituted on one or more benzene ring carbon atoms by short-chained saturated and unsaturated aliphatic radicals (e. g., methyl, ethyl, propyl, butyl, octyl, ethenyl, propenyl, octenyl, etc.). It is preferred that there be not more than 4 substituent groups on the ring and that these substituents contain a total of not more than 16 carbon atoms.

Examples of 2-thio-thiazoles are: 2-mercaptop-benzothiazole; 2-mercaptop-5-methyl thiazole; 2-mercaptop-5-ethyl thiazole; 2-mercaptop-4-methyl thiazole; 2-mercaptop-4,5-dimethyl thiazole; 2-mercaptop-4-ethyl thiazole; 2-mercaptop-4,5-diethyl thiazole; phenyl mercapto-benzothiazole, and methyl mercapto-benzothiazole.

The formaldehyde may be used as such in the reaction, that is, the gaseous formaldehyde, or the aqueous solution of formaldehyde may be used; or compounds which yield formaldehyde, such as paraformaldehyde, may be used in the reaction.

The alkyl groups of the alkyl phenol may be saturated and unsaturated aliphatic groups having from 1 to 24 carbon atoms. The alkyl phenol may have more than 1 alkyl group substituted thereon. It is preferred that the alkyl groups have a total of not more than 32 carbon atoms. Because of the greater effectiveness obtained in the final condensation product as a reactant, it is preferred to use an alkyl phenol containing 1 alkyl group, said alkyl group containing not more than 18 carbon atoms, preferably from 12 to 18 carbon atoms.

Examples of alkyl groups are: methyl, ethyl, propyl, isopropyl, butyl, tertiary-butyl, amyl, tertiary-amyl, octyl, dodecyl, tetradecyl, hexadecyl, octadecyl, butenyl, octenyl, dodecenyl,

tetradecenyl, octadecenyl, butenyl polymers containing from 12 to 16 carbon atoms, etc.

Examples of alkyl phenols are the following: methyl phenol, di-methyl phenol, tri-methyl phenol, iso-propyl phenol, ethyl phenol, di-ethyl phenol, butyl phenol, tertiary-butyl phenol, amyl phenol, di-amyl phenol, tri-amyl phenol, octyl phenol, methyl-octyl phenol, dodecyl phenol, octadecyl phenol, vinyl phenol, butenyl phenol, octadecenyl phenol, polybutylene phenol, wherein the polybutylene group contains from 12 to 16 carbon atoms, condensed ring phenols (such as naphthol and hydroxy anthracene), etc.

The silver protective agents of this invention are effective when they are present in amounts as low as about 0.001% (by weight of total composition). Certain of these compounds have only limited solubility in the lubricating oil and are effective at that solubility. When the protective agents have sufficient solubility, they are effective when each one is used in amounts as great as 5.0%. However, it is preferred that the silver protective agents of this invention be used in amounts sufficient substantially to reduce the corrosion of silver. For example, it is preferred to use these agents in amounts of from about 0.30% to about 1.0%. The major portion of the lubricating composition of this invention is the base oil.

Suitable base oils include a wide variety of lubricating oils such as naphthenic base, paraffin base, and mixed base mineral oils, other hydrocarbon lubricants, e. g., lubricating oil derived from coal products, and synthetic oils, e. g., alkylene polymers (such as polymers of propylene, butylene, etc., and mixtures thereof), alkylene oxide-type polymers, dicarboxylic acid esters and liquid esters of acids of phosphorus. Synthetic oils of the alkylene-oxide type polymer which may be used include those exemplified by the alkylene oxide polymers (e. g., propylene oxide polymers) and derivatives, including alkylene oxide polymers prepared by polymerizing alkylene oxides, e. g., propylene oxide, in the presence of water or alcohols, e. g., ethyl alcohol, and esters of alkylene oxide type polymers, e. g., acetylated propylene oxide polymers prepared by acetylating propylene oxide polymers containing hydroxyl groups.

Synthetic oils of the dicarboxylic acid ester type include those which are prepared by esterifying such dicarboxylic acids as adipic acid, azelaic acid, suberic acid, sebatic acid, alkenyl succinic acid, fumaric acid, maleic acid, etc., with alcohols such as butyl alcohol, hexyl alcohol, 2-ethyl-hexyl alcohol, dodecyl alcohol, etc. Examples of dicarboxylic acid ester synthetic oils include di-butyl adipate, di-hexyl adipate, di-2-ethyl-hexyl sebacate, di-n-hexyl fumarate polymer, etc.

Synthetic oils of the type of liquid esters of the acids of phosphorus include the esters of phosphoric acid, e. g., tricresyl phosphate; the esters of phosphonic acid, e. g., di-ethyl ester of decane phosphonic acid (or other such esters as obtained by reacting alkyl phosphonyl chlorides with hydroxyl-containing compounds such as phenols and aliphatic alcohols, and with olefin oxides such as propylene oxide, as described in Jensen et al. U. S. patent application No. 86,856, now abandoned).

The improved lubricant of the present invention is used wherever elemental sulfur or sulfur compounds containing active sulfur attack metals and are "severely corrosive" to metals which

are being lubricated. Thus, as a result of the present invention, lubricants which normally are "severely corrosive" to metal parts due to attack by sulfur or active sulfur compounds may now be used without fear of corrosion by incorporating therein a condensation product of a 2-thio-thiazole, formaldehyde and an alkyl phenol. "Severely corrosive" is defined as that corrosion which causes a weight loss greater than 30 milligrams in the "silver strip" test noted hereinbelow.

In order to evaluate the agents of this invention for inhibiting corrosion due to active sulfur, a "silver strip corrosion test" was made on numerous agents of this invention. This silver strip corrosion test was performed as follows:

A silver metal strip having the dimensions of 2½ inches by ¾ inch by ½ inch was first cleaned with a wire brush until the strip was highly polished. The strip was weighed and the weight recorded. This highly polished silver strip was then placed in a 600 milliliter beaker in such a manner that the strip was completely immersed when 300 grams of the oil being tested was poured into the beaker. The oil was stirred at a temperature of 300° F. for 20 hours, at which time the silver strip was removed and cleaned, first with chloroform, then with petroleum ether. The appearance of the strip was noted. Those strips which had been severely attacked were quite black. The tested silver strip was washed in 15% aqueous solution of potassium cyanide for about 5 minutes to remove the sulfide film adhering to the strip. After the strip had been washed with potassium cyanide and dried, it was weighed. The difference in weight of the original strip and the strip after the potassium cyanide wash was noted and recorded as the weight loss due to corrosion by the sulfur compound.

The agents of this invention are especially effective as protective agents for silver. However, the protective agents of this invention are also effective in protecting other sulfur-sensitive metals from sulfur attack. Such other sulfur-sensitive metals include copper, aluminum, and alloys of copper and aluminum.

As illustrative of various sulfur-containing extreme pressure agents, detergents, oxidation inhibitors, etc., which cause oils containing them to be severely corrosive to silver, the following may be mentioned: sulfurized lubricating oils, xanthate esters, chlorinated xanthate esters, dialkyl disulfides, sulfurized fatty oils, metal salts of reaction products of olefins and phosphorus pentasulfide, organic trisulfides, tetrasulfides and pentasulfides (e. g., paraffin wax polysulfide), polyvalent metal salts of organo-substituted acids of phosphorus (e. g., zinc hexyl-dithiophosphate), sulfurized olefins (e. g., sulfurized terpene), xanthic acid derivatives (e. g., dibutyl xanthogen disulfide), etc.

Some of the above-indicated additives are more vigorous in their attack on silver than others, and consequently such attack is more difficult to minimize. However, the silver-protective agents are advantageously used even with the more active sulfur additives.

The silver protective agents of this invention are also effective in reducing attack on silver by the sulfur in lubricating oils derived from some of the crude oils characterized by their high sulfur content.

Although the silver protective agents are espe-

cially desirable and preferably used in combination with lubricating oils containing the polyvalent metal salts of organo-substituted thiocarboxylic acids of phosphorus (e. g., zinc cetyl phenyl dithiophosphate), they may be used in lubricating oils also containing such compounds as phenates (e. g., calcium cetyl phenate), sulfonates (e. g., calcium petroleum sulfonate), phosphates (e. g., calcium cetyl phosphate), phenols (e. g., 2,6-di-tertiary-butyl-4-methyl phenol), phosphonates (e. g., calcium white oil phosphonate), thiophosphonates (e. g., calcium cetyl thiophosphonate), etc.

The silver-protective agents of this invention may be added to lubricating compositions containing other agents than sulfur-active agents, that is, other agents which are advantageously present as oiliness agents, blooming agents, viscosity index improvers, pour point depressants, peptizing agents, etc.

Table I below presents data obtained in the "silver strip test" and shows the remarkable effects which the reaction product of Example I hereinbelow (the product obtained by reacting together 2-mercapto-benzothiazole, formaldehyde and an alkyl phenol) as silver-protective agents has in reducing the attack on silver by a California solvent-refined S. A. E. 30 paraffinic base oil containing sulfurized calcium cetyl phenate, sulfurized diparaffin sulfide, calcium petroleum sulfonate and zinc cetyl phenyl dithiophosphate.

Table I

|   | Amount of Protective Agent used in Lubricating Oil (percent by weight) | Silver Strip Test Weight Loss in Milligrams |
|---|------------------------------------------------------------------------|---------------------------------------------|
| 1 |                                                                        | 49.3                                        |
| 2 | 0.1                                                                    | 20.5                                        |
| 3 | 0.2                                                                    | 26.3                                        |
| 4 | 0.3                                                                    | 28.9                                        |
| 5 | 0.8                                                                    | 12.2                                        |
| 6 | 1.0                                                                    | 6.7                                         |

Table II presents data obtained in the "silver strip test" of a California solvent-refined S. A. E. 30 paraffinic base oil to which has been added calcium petroleum sulfonate, sulfurized calcium cetyl phenate and zinc cetyl phenyl di-thiophosphate (using the same protective agent as in above Table I).

Table II

|   | Amount of Protective Agent used in Lubricating Oil (percent by weight) | Silver Strip Test Weight Loss in Milligrams |
|---|------------------------------------------------------------------------|---------------------------------------------|
| 1 |                                                                        | 38.1                                        |
| 2 | 0.3                                                                    | 19.8                                        |
| 3 | 0.4                                                                    | 11.0                                        |
| 4 | 0.5                                                                    | 7.4                                         |
| 5 | 1.0                                                                    | 4.8                                         |

Table III presents data showing the remarkable effectiveness of the compounds of this invention in reducing the severe corrosiveness of a solvent-refined S. A. E. 30 paraffin base oil containing calcium petroleum sulfonate, sulfurized diparaffin sulfide, a barium dithiophosphate and tri-octyl thiophosphate (using the same protective agent as in above Table I).

7  
Table III

|    | Amount of Protective Agent used in Lubricating Oil (percent by Weight) | Silver Strip Test Weight Loss in Milligrams |
|----|------------------------------------------------------------------------|---------------------------------------------|
| 1. |                                                                        | 652.1                                       |
| 2. | 1.0                                                                    | 87.3                                        |

Table IV presents data obtained in the "silver strip test" and shows the remarkable effects which the reaction product of Example II herein below (the product obtained by reacting together 2-mercapto-benzothiazole, formaldehyde and p-tertiary-amyl phenol) as silver protective agent has in reducing the attack of silver of a California solvent-refined S. A. E. 30 paraffinic base oil containing sulfurized calcium cetyl phenate, sulfurized diparaffin sulfide, calcium petroleum sulfonate and zinc cetyl phenyl di-thiophosphate.

Table IV

|    | Amount of Protective Agent used in Lubricating Oil (percent by Weight) | Silver Strip Test Weight Loss in Milligrams |
|----|------------------------------------------------------------------------|---------------------------------------------|
| 1. |                                                                        | 49.3                                        |
| 2. | 0.6                                                                    | 3.5                                         |
| 3. | 0.8                                                                    | 4.4                                         |
| 4. | 1.0                                                                    | 4.1                                         |

Table V presents data obtained in the "silver strip test" and shows the effectiveness of the reaction product of Example III herein below (the product obtained by reacting together 2-mercapto-benzothiazole, formaldehyde and p-tertiary-butyl phenol) as silver protective agent in reducing the attack of silver by a California solvent-refined S. A. E. 30 paraffinic base oil containing sulfurized calcium cetyl phenate, sulfurized diparaffin sulfide, calcium petroleum sulfonate and zinc cetyl phenyl di-thiophosphate.

Table V

|    | Amount of Protective Agent used in Lubricating Oil (percent by Weight) | Silver Strip Test Weight Loss in Milligrams |
|----|------------------------------------------------------------------------|---------------------------------------------|
| 1. |                                                                        | 49.3                                        |
| 2. | 0.8                                                                    | 8.1                                         |

The following examples are presented to illustrate the method of preparing the protective agents of this invention. Although the reactants were used in approximately equimolar amounts, it may be desirable in certain instances to use an excess of one of the reactants in order to obtain greater yields of the condensation product.

*Example I.—Preparation of the condensation product of 2-mercapto-benzothiazole, formaldehyde and a polybutylene alkylated phenol*

The "polybutylene" alkyl group of the phenol of this example was composed of a mixture of polybutylene groups having from 12 to 16 carbon atoms. The hydroxyl number of the polybutylene alkylated phenol was 151.

A mixture of 20.75 grams of 2-mercapto-benzothiazole, 3.75 grams of para-formaldehyde, 46.5

grams of polybutylene alkylated phenol and 2.50 grams of hexamethylene tetramine (used herein as a catalyst) was heated for 40 minutes at a temperature ranging from 105° C. to 130° C. A yellowish-orange colored resinous product was obtained. This product, which has a molecular weight of 560, contained 11.13% sulfur, 2.79% nitrogen, 72.98% carbon and 8.63% hydrogen.

*Example II.—Preparation of the condensation product of 2-mercapto-benzothiazole, formaldehyde and para-tertiary-amyl phenol*

A mixture of 33.4 grams of 2-mercapto-benzothiazole, 33 grams of para-tertiary-amyl phenol, 6 grams of para-formaldehyde and 0.3 gram of hexamethylene tetramine (used herein as a catalyst) was heated for 30 minutes at a temperature ranging from 150° C. to 160° C. A light amber colored resinous product was obtained.

*Example III.—Preparation of condensation product of 2-mercapto-benzothiazole, formaldehyde and para-tertiary-butyl phenol*

A mixture of 84 grams of 2-mercapto-benzothiazole, 75 grams of para-tertiary-butyl phenol, 15 grams of formaldehyde and 1 gram of hexamethylene tetramine (used herein as catalyst) was heated for 45 minutes at a temperature ranging from 150° C. to 160° C. A light amber colored resinous product was obtained.

The data and examples hereinabove show the outstanding effectiveness of the protective agents of this invention in protecting silver from sulfur attack. In addition, the protective agents of this invention also protect silver from selenium attack. That is, lubricants which contain active selenium compounds as additives, for example, dialkyl monoselenides, dialkyl diselenides, dialkyl polyselenides, seleno-mercaptans, metal alkyl selenides, etc., show attack on silver by the selenium. However, the protective agents of this invention inhibit the attack on silver by lubricants containing selenium compounds.

We claim:

1. A lubricant consisting essentially of a major portion of a sulfur-containing lubricating oil composition severely corrosive to silver, and small amounts, sufficient substantially when present in combination to reduce the sulfur attack on silver, of a condensation product obtained by reacting together equal molar proportions of a 2-mercapto-thiazole, formaldehyde and an alkyl phenol wherein the alkyl group is an aliphatic group containing from 12 to 18 carbon atoms at a temperature greater than 105° C. for at least 30 minutes.

2. A lubricant consisting essentially of a major portion of a sulfur-containing lubricating oil composition which is severely corrosive to silver, and added to said sulfur-containing lubricating oil composition, a condensation product obtained by reacting together equal molar proportions of a 2-mercapto-thiazole, formaldehyde and an alkyl phenol wherein the alkyl group is an aliphatic group containing from 12 to 18 carbon atoms at a temperature greater than 105° C. for at least 30 minutes.

3. A lubricating oil composition at least 95% of which is composed of an admixture of an oil of lubricating viscosity and lubricating oil additives having present sulfur, which admixture is corrosive to silver, and compounded with this mixture a condensation product obtained by reacting together equal molar proportions of a 2-mercapto-thiazole, formaldehyde and an alkyl

phenol wherein the alkyl group is an aliphatic group containing from 12 to 18 carbon atoms at a temperature greater than 105° C. for at least 30 minutes.

4. A lubricant consisting essentially of a major portion of a sulfur-containing lubricating oil composition severely corrosive to silver, and small amounts, sufficient substantially when present in combination to reduce the sulfur attack on silver, of a condensation product obtained by reacting together equal molar proportions of a 2-mercapto-thiazole, wherein the 2 adjacent carbon atoms of the thiazole ring form a part of a benzene ring, formaldehyde and an alkyl phenol, wherein the alkyl group is a polybutylene group at a temperature greater than 105° C. for a period of at least 30 minutes.

5. A lubricant consisting essentially of a major portion of a sulfur-containing lubricating oil composition severely corrosive to silver, and small amounts, sufficient substantially when present in combination to reduce the sulfur attack on silver, of a condensation product obtained by reacting together equal molar proportions of 2-mercapto-benzothiazole, formaldehyde and a polybutylene alkylated phenol, wherein the polybutylene group contains from 12 to 16 carbon atoms at a temperature greater than 105° C. for a period of at least 30 minutes.

6. A lubricating oil composition at least 95% of which is composed of an admixture of an oil of lubricating viscosity and lubricating oil additives having present sulfur, which admixture is corrosive to silver, and compounded with this mixture from about 0.4% to about 1% of a condensation product obtained by reacting together equal molar proportions of 2-mercapto-benzothiazole, formaldehyde and a polybutylene alkylated phenol, wherein the polybutylene group contains from 12 to 16 carbon atoms at a temperature

greater than 105° C. for a period of at least 30 minutes.

7. A sulfur-containing lubricating oil severely corrosive to silver, and having in said lubricant a condensation product obtained by reacting together equal molar proportions of a 2-mercapto-thiazole, wherein the 2 adjacent carbon atoms of the thiazole ring carbons form a part of a benzene ring, formaldehyde and an alkyl phenol wherein the alkyl group is an aliphatic group containing from 12 to 18 carbon atoms at a temperature greater than 105° C. for a period of at least 30 minutes.

8. A sulfur-containing lubricating oil severely corrosive to silver, and small amount, sufficient substantially to reduce the sulfur attack on silver, of a condensation product obtained by reacting together equal molar proportions of 2-mercapto-benzothiazole, formaldehyde and a polybutylene alkylated phenol, wherein the polybutylene group contains from 12 to 16 carbon atoms at a temperature greater than 105° C. for a period of at least 30 minutes.

RICHARD L. WOODRUFF.  
WILLIAM T. STEWART.  
WARREN LOWE.

#### REFERENCES CITED

The following references are of record in the file of this patent:

#### UNITED STATES PATENTS

| Number    | Name         | Date          |
|-----------|--------------|---------------|
| 2,154,096 | Loane        | Apr. 11, 1939 |
| 2,201,258 | Busse        | May 21, 1940  |
| 2,318,629 | Prutton      | May 11, 1943  |
| 2,334,594 | Zimmer       | Nov. 16, 1943 |
| 2,384,002 | Bayes        | Sept. 4, 1945 |
| 2,414,257 | Evans et al. | Jan. 14, 1947 |